



US010144995B2

(12) **United States Patent**  
Lin et al.

(10) **Patent No.:** US 10,144,995 B2  
(45) **Date of Patent:** Dec. 4, 2018

(54) **MIXED MAGNETIC POWDERS AND THE ELECTRONIC DEVICE USING THE SAME**

(71) Applicant: **CYNTEC CO., LTD.**, Hsinchu (TW)

(72) Inventors: **Lu-Kuei Lin**, New Taipei (TW);  
**Shih-Feng Chien**, Hsinchu County (TW); **Po-I Wu**, Taipei (TW)

(73) Assignee: **CYNTEC CO., LTD.**, Hsinchu (TW)

(\*) Notice: Subject to any disclaimer, the term of this patent is extended or adjusted under 35 U.S.C. 154(b) by 0 days.

(21) Appl. No.: **15/989,206**

(22) Filed: **May 25, 2018**

(65) **Prior Publication Data**

US 2018/0274068 A1 Sep. 27, 2018

**Related U.S. Application Data**

(63) Continuation of application No. 15/603,460, filed on May 24, 2017, now Pat. No. 10,006,110, which is a continuation of application No. 14/693,956, filed on Apr. 23, 2015, now Pat. No. 9,719,159.

(60) Provisional application No. 62/079,573, filed on Nov. 14, 2014, provisional application No. 62/054,388, filed on Sep. 24, 2014.

(51) **Int. Cl.**

**H01F 27/00** (2006.01)  
**C22C 38/32** (2006.01)  
**C22C 38/34** (2006.01)  
**C22C 45/02** (2006.01)  
**H01F 5/00** (2006.01)  
**H01F 27/24** (2006.01)

**C22C 38/00** (2006.01)

**B22F 1/00** (2006.01)

**C22C 38/02** (2006.01)

**C22C 33/02** (2006.01)

**H01F 1/153** (2006.01)

**H01F 17/04** (2006.01)

(52) **U.S. Cl.**

CPC ..... **C22C 38/32** (2013.01); **B22F 1/00** (2013.01); **B22F 1/0014** (2013.01); **C22C 33/0264** (2013.01); **C22C 38/002** (2013.01); **C22C 38/02** (2013.01); **C22C 38/34** (2013.01); **C22C 45/02** (2013.01); **H01F 1/153** (2013.01); **H01F 1/15375** (2013.01); **H01F 5/00** (2013.01); **H01F 17/04** (2013.01); **H01F 27/00** (2013.01); **H01F 27/24** (2013.01); **C22C 2200/02** (2013.01); **C22C 2202/02** (2013.01); **H01F 2017/048** (2013.01)

(58) **Field of Classification Search**

CPC ..... H01F 27/00–27/36

USPC ..... 336/65, 83, 200, 232–234

See application file for complete search history.

*Primary Examiner* — Tuyen Nguyen

(74) *Attorney, Agent, or Firm* — Ming-Lee Teng; Litron Patent & Trademark Office

(57) **ABSTRACT**

Mixed magnetic powders for making a magnetic core or body is disclosed, wherein the mixed magnetic powders comprises a first magnetic powder and a second magnetic powder, each of the first magnetic powder and the second magnetic powder being made of a soft magnetic material, wherein the average particle diameter of the first magnetic powder is greater than that of the second magnetic powder, and each of the first magnetic powder and the second magnetic powder has a pre-configured particle size distribution for increasing the density of the magnetic body.

**20 Claims, 8 Drawing Sheets**





Fig. 1



Fig. 2



Fig. 3



Fig. 4



Fig. 5



Fig. 6



Fig. 7



Fig. 8

## 1

## MIXED MAGNETIC POWDERS AND THE ELECTRONIC DEVICE USING THE SAME

## CROSS-REFERENCES TO RELATED APPLICATIONS

This application is a continuation of U.S. patent application Ser. No. 15/603,460 filed on May 24, 2017, which is a continuation of U.S. patent application Ser. No. 14/693,956 filed on Apr. 23, 2015, which claims the benefit of U.S. Provisional Patent Application No. 62/054,388 filed on Sep. 24, 2014 and 62/079,573 filed on Nov. 14, 2014, which are hereby incorporated by reference herein and made a part of the specification.

## BACKGROUND OF THE INVENTION

## I. Field of the Invention

The present invention relates to mixed powders for manufacturing an electronic component, and in particular, to mixed magnetic powders for manufacturing an inductive component.

## II. Description of Related Art

As technology advances, inductive components have become smaller and smaller with lower power consumption especially when operating at high frequency. Conventionally, different magnetic powders are mixed to form a magnetic body or a magnetic core by a pressure molding process for making an inductive component. The magnetic powders can be made of a soft magnetic material and the soft magnetic powders can be mixed with an adhesive material, after which the mixture of the magnetic powders and the adhesive material will undergo a molding process to form a magnetic body or a magnetic core.

In general, the higher the pressure in the molding process, the higher the core bulk density and the permeability of the core. However, if the pressure is too high, it will cause damage of the internal insulating material or residual stress which will induce the deformation of the magnetic core; therefore, the pressure can only increase the core bulk density and the permeability of the core to a certain limit.

Furthermore, conventional magnetic powders are mixed together with a single particle size distribution or different hardness between different magnetic powders, which has reached a limit for increasing the bulk density of the magnetic body or the magnetic core. Therefore, how to improve both the core bulk density and the initial permeability without higher pressure is a desired goal in the industry.

## SUMMARY OF THE INVENTION

The present invention provides a soft magnetic material with mixed magnetic powders having a distribution of various particle sizes to form a magnetic body or a magnetic core with a higher bulk density and a permeability.

In one embodiment, mixed magnetic powders for making a magnetic core or body is disclosed, wherein the mixed magnetic powders comprises: a first magnetic powder; a second magnetic powder, wherein the first magnetic powder and the second magnetic powder are made of a same soft magnetic material, wherein the ratio of the D50 of the first magnetic powder to the D50 of the second magnetic powder is in the range of 5 to 12, wherein the first magnetic powder

## 2

weighs 50 to 90 percent of the total weight of the first magnetic powder and the second magnetic powder; and the second magnetic powder weighs 10 to 50 percent of the total weight of the first magnetic powder and the second magnetic powder.

In one embodiment, the mixed magnetic powders according to claim 1, wherein the mixed magnetic powders are made of amorphous alloy powder.

In one embodiment, the Nano-indentation hardness of the amorphous alloy powder is not less than 7 Gpa.

In one embodiment, the ratio of the D50 of the first magnetic powder to the D50 of the second magnetic powder is in the range of 6 to 9.

In one embodiment, the ratio of the D50 of the first magnetic powder to the D50 of the second magnetic powder is in the range of 10 to 12.

In one embodiment, the first magnetic powder weighs 80 percent of the total weight of the first magnetic powder and the second magnetic powder; and the second magnetic powder weighs 20 percent of the total weight of the first magnetic powder and the second magnetic powder.

In one embodiment, the first magnetic powder weighs 70 percent of the total weight of the first magnetic powder; and the second magnetic powder and the second magnetic powder weighs 30 percent of the total weight of the first magnetic powder and the second magnetic powder.

In one embodiment, the mixed magnetic powders are made of amorphous alloy powder, wherein the weight ratio of the first magnetic powder and the second magnetic powder is 6:4 when the ratio of the D50 of the first magnetic powder to the D50 of the second magnetic powder is greater than 8.97, and the weight ratio of the first magnetic powder and the second magnetic powder is 7:3 when the ratio of the D50 of the first magnetic powder to the D50 of the second magnetic powder is less than 8.97.

In one embodiment, the D50 of the first magnetic powder is in the range of 17 to 36 um and the D50 of the second magnetic powder is in the range of 1.0 to 3.5 um.

In one embodiment, the D50 of the first magnetic powder is in the range of 20 to 34 um and the D50 of the second magnetic powder is in the range of 1.8 to 3.2 um.

In one embodiment, the D50 of the first magnetic powder is in the range of 17 to 20 um and the D50 of the second magnetic powder is in the range of 1.0 to 1.8 um.

In one embodiment, the D50 of the first magnetic powder is in the range of 17 to 36 um and the D50 of the second magnetic powder is in the range of 1.0 to 3.5 um; the D10 of the first magnetic powder is in the range of 8 to 26 um and the D10 of the second magnetic powder is in the range of 0.5 to 1.7 um; and the D90 of the first magnetic powder is in the range of 30 to 52 um and the D90 of the second magnetic powder is in the range of 2.8 to 5.6 um.

In one embodiment, the D50 of the first magnetic powder is in the range of 20 to 34 um and the D50 of the second magnetic powder is in the range of 1.8 to 3.2 um; the D10 of the first magnetic powder is in the range of 10~23 um and the D10 of the second magnetic powder is in the range of 1~1.7 um; and the D90 of the first magnetic powder is in the range of 36~52 um and the D90 of the second magnetic powder is in the range of 3.5 to 5.6 um.

In one embodiment, the D50 of the first magnetic powder is in the range of 17 to 20 um and the D50 of the second magnetic powder is in the range of 1.0 to 1.8 um; the D10 of the first magnetic powder is in the range of 8~10 um and the D10 of the second magnetic powder is in the range of 0.5~1.0 um; and the D90 of the first magnetic powder is in

the range of 30~36  $\mu\text{m}$  and the D90 of the second magnetic powder is in the range of 2.8 to 3.5  $\mu\text{m}$ .

In one embodiment, the ratio of the number of particles of the first magnetic powder at D50 to the number of particles of the first magnetic powder at D10 is greater than 2 and the ratio of the number of particles of the first magnetic powder at D50 to the number of particles of the first magnetic powder at D90 is greater than 1, and wherein the ratio of the number of particles of the second magnetic powder at D50 to the number of particles of the second magnetic powder at D10 is greater than 2 and the ratio of the number of particles of the second magnetic powder at D50 to the number of particles of the second magnetic powder at D90 is greater than 1.

In one embodiment, the ratio of the D50 of the first magnetic powder to the D50 of the second magnetic powder is in the range of 10 to 12, wherein the ratio of the number of particles of the first magnetic powder at D50 to the number of particles of the first magnetic powder at D10 is greater than 3 and the ratio of the number of particles of the first magnetic powder at D50 to the number of particles of the first magnetic powder at D90 is greater than 1.5, and wherein the ratio of the number of particles of the second magnetic powder at D50 to the number of particles of the second magnetic powder at D10 is greater than 3 and the ratio of the number of particles of the second magnetic powder at D50 to the number of particles of the second magnetic powder at D90 is greater than 1.3.

In one embodiment, the mixed magnetic powders are made of iron powders.

In one embodiment, the mixed magnetic powders are made of amorphous alloy powder, wherein the first magnetic power comprises 0.5~1 wt % C, 6.2~7.2 wt % Si, 0~3.0 wt % Cr, 2.2~2.8 wt % B, and the rest is Fe, wherein 0% is less than 5000 ppm, and wherein the second magnetic power comprises 0.5~1 wt % C, 5.7~7.7 wt % Si, 0~3.0 wt % Cr, 2.0~3.0 wt % B, and the rest is Fe, wherein 0% is less than 10000 ppm.

In one embodiment, a method to produce a magnetic core or body is disclosed, the method comprising: forming a first magnetic powder and a second magnetic powder, wherein the first magnetic powder and the second magnetic powder are made of the same material, wherein the mean particle diameter of the first magnetic powder is greater than the mean particle diameter of the second magnetic powder, wherein the ratio of the D50 of the first magnetic powder to the D50 of the second magnetic powder is in the range of 5 to 12, wherein the ratio of the number of particles of the first magnetic powder at D50 to the number of particles of the first magnetic powder at D10 is greater than 2 and the ratio of the number of particles of the first magnetic powder at D50 to the number of particles of the first magnetic powder at D90 is greater than 1, and wherein the ratio of the number of particles of the second magnetic powder at D50 to the number of particles of the second magnetic powder at D10 is greater than 2 and the ratio of the number of particles of the second magnetic powder at D50 to the number of particles of the second magnetic powder at D90 is greater than 1; mixing the first magnetic powder and the second magnetic powder with an adhesive material, wherein the weight of the adhesive material is 1 to 5 percent of the total weight of the first magnetic powder and the second magnetic powder; and performing a pressure molding process to the mixture of the first magnetic powder, the second magnetic powder and the adhesive material to form the magnetic core.

In one embodiment, the adhesive material is thermoset resin.

In one embodiment, the first magnetic powder and the second magnetic powder are made of amorphous alloy, and the nano-indentation hardness of the amorphous alloy is not less than 7 Gpa.

In one embodiment, the pressure is between 0.5 t/cm<sup>2</sup> to 4 t/cm<sup>2</sup>.

In one embodiment, the mixed magnetic powders are made of amorphous alloy powder, wherein the first magnetic power comprises 0.5~1 wt % C, 6.2~7.2 wt % Si, 0~3.0 wt % Cr, 2.2~2.8 wt % B, and the rest is Fe, wherein 0% is less than 5000 ppm, and wherein the second magnetic power comprises 0.5~1 wt % C, 5.7~7.7 wt % Si, 0~3.0 wt % Cr, 2.0~3.0 wt % B, and the rest is Fe, wherein 0% is less than 10000 ppm.

The present invention provides an electronic device, comprising: a magnetic body, comprising: a first magnetic powder; a second magnetic powder, wherein the first magnetic powder and the second magnetic powder are made of a same soft magnetic material, wherein the ratio of the D50 of the first magnetic powder to the D50 of the second magnetic powder is in the range of 5 to 12, wherein the first magnetic powder weighs 60 to 90 percent of the total weight of the first magnetic powder and the second magnetic powder and the second magnetic powder weighs 10 to 40 percent of the total weight of the first magnetic powder and the second magnetic powder, an adhesive material, joining the first magnetic powder and the second magnetic powder; and a wire. According to one embodiment of the present invention, a wire includes a buried part buried in the magnetic body or a winding part winding on the magnetic body. According to one embodiment of the present invention, the magnetic body is manufactured by a molding process, and the molding pressure of the molding process is 6t/cm<sup>2</sup>~11t/cm<sup>2</sup>. In one embodiment, the molding pressure of the molding process is 6t/cm<sup>2</sup>~11t/cm<sup>2</sup>.

In one embodiment, the corresponding optimum weight ratio of the first magnetic powder and second magnetic powder is 7:3. As a result, for a given the D50 ratio of the first magnetic powder and second magnetic powder, the corresponding optimum weight ratio of the first magnetic powder and second magnetic powder can be found to produce the magnetic body to a achieve a higher bulk density and a higher initial permeability.

In order to make the aforementioned and other features and advantages of the present invention more comprehensible, several embodiments accompanied with figures are described in detail below.

#### BRIEF DESCRIPTION OF THE DRAWINGS

The accompanying drawings are included to provide a further understanding of the invention, and are incorporated in and constitute a part of this specification. The drawings illustrate embodiments of the invention and, together with the description, serve to explain the principles of the invention.

FIG. 1 is a cross-sectional view illustrating the micro-structure of the soft magnetic material according to one embodiment of the present invention.

FIG. 2 is a cross-sectional view illustrating the micro-structure of the soft magnetic material according to another embodiment of the present invention.

FIG. 3 is a cross-sectional view of the magnetic body made of the soft magnetic material according to one embodiment of the present invention.

FIG. 4 is a cross-sectional view of the magnetic body with an embedded coil according to one embodiment of the present invention.

FIG. 5 and FIG. 6 illustrate the impacts of the weight ratio of a first magnetic powder and a second magnetic powder.

FIG. 7 shows the Q factor vs the frequencies of an inductor made by the present invention compared with conventional technology.

FIG. 8 shows the inductance vs the frequencies of the inductor made by the present invention compared with conventional technology.

#### DESCRIPTION OF EMBODIMENTS

For the following description D10, D50 and D90 are used for describing the particle size distribution of magnetic powders. D10 means 10% of the total number of the particles is less than the D10, D50 means 50% of the total number of the particles is less than D50 and D90 means 90% of the total number of the particles is less than D90.

FIG. 1 depicts an enlarged view of the microstructure of a soft magnetic material according to one embodiment of the present invention. Please refer to FIG. 1, the soft magnetic material comprises a first magnetic powder 10 and a second magnetic powder 20, wherein the average particle diameter of the first magnetic powder 10 is greater than the average particle diameter of the second magnetic powder 20, wherein the ratio of the D50 of the first magnetic powder to the D50 of the second magnetic powder is in the range of 5 to 12, wherein the ratio of the number of particles of the first magnetic powder at D50 to the number of particles of the first magnetic powder at D10 is greater than 2 and the ratio of the number of particles of the first magnetic powder at D50 to the number of particles of the first magnetic powder at D90 is greater than 1, and wherein the ratio of the number of particles of the second magnetic powder at D50 to the number of particles of the second magnetic powder at D10 is greater than 2 and the ratio of the number of particles of the second magnetic powder at D50 to the number of particles of the second magnetic powder at D90 is greater than 1. Preferably, the ratio of the D50 of the first magnetic powder to the D50 of the second magnetic powder is in the range of 6 to 9, wherein the ratio of the number of particles of the first magnetic powder at D50 to the number of particles of the first magnetic powder at D10 is greater than 3 and the ratio of the number of particles of the first magnetic powder at D50 to the number of particles of the first magnetic powder at D90 is greater than 1.5, and wherein the ratio of the number of particles of the second magnetic powder at D50 to the number of particles of the second magnetic powder at D10 is greater than 3 and the ratio of the number of particles of the second magnetic powder at D50 to the number of particles of the second magnetic powder at D90 is greater than 1.3. Most preferably, the ratio of the D50 of the first magnetic powder to the D50 of the second magnetic powder is in the range of 10 to 12, wherein the ratio of the number of particles of the first magnetic powder at D50 to the number of particles of the first magnetic powder at D10 is greater than 3 and the ratio of the number of particles of the first magnetic powder at D50 to the number of particles of the first magnetic powder at D90 is greater than 1.5, and wherein the ratio of the number of particles of the second magnetic powder at D50 to the number of particles of the second magnetic powder at D10 is greater than 3 and the ratio of the number of particles of the second magnetic powder at D50 to the number of particles of the second magnetic powder at D90 is greater than 3 and the ratio of the number of particles of the second magnetic powder at D50 to the number of particles of the second magnetic powder at D10 is greater than 1, which means (Qd50/Qd10) is greater than 1 for the second magnetic powder.

the second magnetic powder at D50 to the number of particles of the second magnetic powder at D90 is greater than 1.3.

In one embodiment, the weight ratio of the first magnetic powder 10 and the second magnetic powder 20 is 9:1, which means the first magnetic powder 10 has 90% of the total weight of the mixed magnetic powders, and the second magnetic powder 20 has 10% of the total weight of the mixed magnetic powders. Preferably, the weight ratio of the first magnetic powder 10 and the second magnetic powder 20 is 8:2, which means the first magnetic powder 10 has 80% of the total weight of the mixed magnetic powders, and the second magnetic powder 20 has 20% of the total weight of the mixed magnetic powders. Most preferably, the weight ratio of the first magnetic powder 10 and the second magnetic powder 20 is 7:3, which means the first magnetic powder 10 has 70% of the total weight of the mixed magnetic powders, and the second magnetic powder 20 has 30% of the total weight of the mixed magnetic powders.

In one embodiment, wherein the D50 of the first magnetic powder is in the range of 17 to 36 um and the D50 of the second magnetic powder is in the range of 1.0 to 3.5 um, the D10 of the first magnetic powder is in the range of 8 to 26 um and the D10 of the second magnetic powder is in the range of 0.5 to 1.7 um, the D90 of the first magnetic powder is in the range of 30 to 52 um and the D90 of the second magnetic powder is in the range of 2.8 to 5.6 um.

Preferably, the D50 of the first magnetic powder is in the range of 20~34 um and the D50 of the second magnetic powder is in the range of 1.8~3.2 um, the D10 of the first magnetic powder is in the range of 10~23 um and the D10 of the second magnetic powder is in the range of 1.0~1.7 um, the D90 of the first magnetic powder is in the range of 36 to 52 um and the D90 of the second magnetic powder is in the range of 3.5 to 5.6 um.

Most preferably, the D50 of the first magnetic powder is in the range of 17~20 um and the D50 of the second magnetic powder is in the range of 1.0~1.8 um, the D10 of the first magnetic powder is in the range of 8~10 um and the D10 of the second magnetic powder is in the range of 0.5 to 1.0 um, the D90 of the first magnetic powder is in the range of 30~36 um and the D90 of the second magnetic powder is in the range of 2.8~3.5 um.

In one embodiment, the particle size distribution of the first magnetic powder and second magnetic powder comprising: the ratio of the number of particles of the first magnetic powder at D50 (Qd50) and the number of particles of the first magnetic powder at D10 (Qd10) is greater than 2, which means (Qd50/Qd10) is greater than 2 for the first magnetic powder, the ratio of the number of particles of the first magnetic powder at D50 (Qd50) and the number of particles of the first magnetic powder at D90 (Qd90) is greater than 1, which means (Qd50/Qd90) is greater than 1 for the first magnetic powder; and the ratio of the number of particles of the second magnetic powder at D50 (Qd50) and the number of particles of the second magnetic powder at D10 (Qd10) is greater than 2, which means (Qd50/Qd10) is greater than 2 for the second magnetic powder, the ratio of the number of particles of the second magnetic powder at D50 (Qd50) and the number of particles of the second magnetic powder at D90 (Qd90) is greater than 1, which means (Qd50/Qd90) is greater than 1 for the second magnetic powder.

Based on the above descriptions, the first magnetic powder 10 and the second magnetic powder 20 can be mixed together according to a weight ratio, wherein the first magnetic powder 10 and the second magnetic powder 20

have a particular particle size distribution such that the second magnetic powder **20** can be easily filled into the spaces between the particles of the first magnetic powder **10**, thereby increasing the bulk density of the mixed magnetic powders compared with conventional technology.

In one embodiment, each of the first material **10** and the second magnetic powder magnetic powder **20** comprises a metal alloy powder. The metal alloy powder can be one of the following: Fe—Cr—Si alloy powder, Fe—Ni alloy powder, amorphous alloy powder, Fe—Si, Fe—Al or other suitable alloy powder.

In one embodiment, the material of each of the first material **10** and the second magnetic powder magnetic powder **20** comprises iron or iron alloy.

In one embodiment, the first magnetic powder **10** and second magnetic powder **20** are made of amorphous alloy powders, and the nano-indentation hardness of amorphous alloy powder is not less than 7 Gpa. Preferably, the first magnetic powder **10** is composed of the following materials expressed by percentage of mass: 0.5 to 1% of carbon (C), 6.2~7.2% of silicon (Si), 0~3.0% of chromium (Cr), 2.2 to 2.8% of boron (B), and the remaining proportion of iron (Fe), where 0% is less than 5000 ppm; the second magnetic powder **20** is composed of the following materials expressed by percentage of mass: 0.5 to 1% of carbon (C), 5.7 to 7.7% of silicon (Si), 0~3.0% of chromium (Cr), 2.0~3.0% of boron (B), and the remaining proportion of iron (Fe), where 0% is less than 10000 ppm.

FIG. 2 depicts an enlarged view of the microstructure of a soft magnetic material according to one embodiment of the present invention. Please refer to FIG. 2, the soft magnetic material comprises the first magnetic powder **10** and the second magnetic powder **20** as described in FIG. 1, and adhesive material **30** mixed with the first magnetic powder **10** and the second magnetic powder **20**, wherein the weight of the adhesive material is 1 to 5 percent of the total weight of the first magnetic powder and the second magnetic powder. The adhesive material **30** may be thermosetting resins such as epoxy resin. Preferably, the first magnetic powder **10** and second magnetic powder **20** are amorphous alloy powders.

In another aspect of the present invention, a method to produce a magnetic body **40** is disclosed, wherein the method comprises: forming a soft magnetic material mixture **M** comprising a first magnetic powder and a second magnetic powder, wherein the first magnetic powder and the second magnetic powder are made of the same material, wherein the mean particle diameter of the first magnetic powder is greater than the mean particle diameter of the second magnetic powder, wherein the ratio of the D50 of the first magnetic powder to the D50 of the second magnetic powder is in the range of 5 to 12, wherein the ratio of the number of particles of the first magnetic powder at D50 to the number of particles of the first magnetic powder at D10 is greater than 2 and the ratio of the number of particles of the first magnetic powder at D50 to the number of particles of the first magnetic powder at D90 is greater than 1, and wherein the ratio of the number of particles of the second magnetic powder at D50 to the number of particles of the second magnetic powder at D10 is greater than 2 and the ratio of the number of particles of the second magnetic powder at D50 to the number of particles of the second magnetic powder at D90 is greater than 1; mixing the first magnetic powder and the second magnetic powder with an adhesive material, wherein the weight of the adhesive material is 1 to 5 percent of the total weight of the first magnetic powder and the second magnetic powder; and performing a

pressure molding process to the mixture of the first magnetic powder, the second magnetic powder and the adhesive material to form a magnetic body **40**, as shown in FIG. 3.

In one embodiment, the molding pressure is 0.1 tons per square centimeter to 6 tons per square. In one embodiment, the method includes a heating process at a temperature 300° C.

FIG. 3 depicts a sectional view of a magnetic body **40** which has a higher bulk density by using the mixture of the soft magnetic material **M** with a particular particle size distribution of magnetic powders, wherein a pressure molding process is applied to the mixture of the soft magnetic material **M** to form a magnetic body **40**, whereby the initial permeability can be enhanced compared with conventional technology. The magnetic body **40** can be used as a magnetic core of an inductive component having a higher permeability, lower power consumption and lower core loss compared with conventional technology. On the other hand, if the magnetic body **40** is targeted to a given bulk density, the pressure for molding the soft magnetic material **M** can be reduced compared with conventional technology for producing the same bulk density.

FIG. 4 depicts a sectional view of a magnetic body **40** which is made by using the mixture of the soft magnetic material **M** and a coil **50** embedded in the mixture of the soft magnetic material through a pressure molding process. Inductor **L** is made of a sectional structure view of one embodiment, the coil **50** is made of enameled wire having an insulating outer layer, and since the soft magnetic material of the present invention has a higher bulk density, the molding pressure to form the magnetic material **40** can be reduced compared with the conventional mixed powders, thereby preventing damage or deformation of the magnetic body **40** during the pressure molding process.

Based on the above descriptions, the magnetic body made of the mixture of the soft magnetic material **M** has the following advantages compared with conventional technology: (1) since the D50 of the each of the first and the second magnetic powder is smaller, it can decrease eddy current loss; (2) since the first and the second magnetic powder have a particular particle size distribution, it can achieve a higher bulk density; (3) the molding pressure to form the magnetic material **40** can be reduced for a given bulk density produced by conventional technology, thereby preventing damage or deformation of the magnetic body during the pressure molding process. In addition, if the amorphous alloy powder with a greater hardness is used for the first and the second magnetic powder, it can reduce the residual stress during molding, thereby reducing the coercive force and the magnetic losses.

The following experiments are carried out for demonstrating the technical features, effects and advantages described above.

The experiment I shows the particle size distributions of the first magnetic powder **10** and the second magnetic powder **20** as described above that impacts the bulk density, energy loss, and other characteristic of the magnetic body.

Table 1 shows the bulk density, energy loss, and other characteristic of the magnetic body according to the experiment I.

Under the condition that the D50 of the second magnetic powder **20** is fixed at 3.21  $\mu$ m, Table 1 shows that the weight ratio of the first magnetic powder **10** and second magnetic powder **20** is 6:4 in case 1. As shown in cases 2, 3, 4, when the D50 of the first magnetic powder **10** is reduced from 33.5  $\mu$ m of the case 1 to 28.8  $\mu$ m of the case 2, 20.4  $\mu$ m of the case 3, 17.6  $\mu$ m of the case 4, the high-frequency loss  $P_{cv}$  (1

MHz/20 mT) is reduced to 701.4 kw/m<sup>3</sup>, 664.8 kw/m<sup>3</sup> and 643.8, 607.5 kw/m<sup>3</sup> in cases 2, 3 and 4, respectively, because when the D50 of the first magnetic powder **10** is reduced, the eddy current will be reduced, thereby reducing the high-frequency loss. However, when the D50 of the first magnetic powder **10** is reduced in cases 2, 3, and 4 compared with that of the case 1, the density of magnetic body will be decreased from 5.66 g/cm<sup>3</sup> of case 1, to 5.63 g/cm<sup>3</sup>, 5.62 g/cm<sup>3</sup> and 5.38 g/cm<sup>3</sup> in cases 2, 3 and 4, respectively, which resulting in a lower initial permeability rate from 28.5 of case 1 to 27.6, 26.2 and 21.8 in cases 2, 3 and 4, respectively, while the low-frequency energy loss Pcv (100 KHz/20 mT) increased from 31.8 kw/m<sup>3</sup> of case 1 to 32.4, 36.1 and 42 kw/m<sup>3</sup> in cases 2, 3 and 4, respectively, due to the fact that the permeability is reduced when the D50 of the first magnetic powder **10** is reduced causing higher hysteresis loss. As a result, as the D50 of the first magnetic powder **10** is reduced, the weight ratio of the first magnetic powder and second magnetic powder should be adjusted to increase the bulk density and the permeability.

Please note that, in the following Table 1, 2 and 3, “L\*” represents “Large powder” or the first magnetic powder; “S\*\*” represents “Small powder” or the second magnetic powder; “D\*” represents Density; “L\*/S\*/Wt Ratio” represents the weight ratio of the large power to the small power; “Ad\*wt %” represents “weight percentage of Adhesive material”; “P” represents “Pressure” and “initial Perm” represents “initial permeability”; Pcv\*represents (kw/m<sup>3</sup>) 100 kHz/20 mT and Pcv\*\*represents (kw/m<sup>3</sup>) 1 MHz/20 mT.

As shown in Table 2, as the D50 ratio of the first magnetic powder **10** and second magnetic powder **20** (that is, D50 of the first magnetic powder/D50 of the second magnetic powder) changes, the optimum weight ratio of the first magnetic powder **10** and the second magnetic powder **20** also changes.

FIG. 5 and FIG. 6 illustrate the corresponding optimum weight ratio of the first magnetic powder **10** and second magnetic powder **20** as the D50 ratio of the first magnetic powder **10** and second magnetic powder **20** changes. As shown in FIG. 5 and FIG. 6, when the D50 ratio of the first magnetic powder **10** and second magnetic powder **20** is greater than 8.97, the corresponding optimum weight ratio of the first magnetic powder **10** and second magnetic powder is 6:4; when the D50 ratio of the first magnetic powder **10** and second magnetic powder **20** is less than 8.97, the corresponding optimum weight ratio of the first magnetic powder **10** and second magnetic powder is 7:3. As a result, for a given D50 ratio of the first magnetic powder **10** and second magnetic powder **20**, the corresponding optimum weight ratio of the first magnetic powder **10** and second magnetic powder **20** can be found to produce the magnetic body **40** to achieve a higher bulk density and a higher initial permeability, wherein the initial permeability can be maintained between 27 to 28, while keeping the low-energy loss variation small as the hysteresis loss is not worsened too much. It is worth noting that, even the D50 of the first magnetic powder **10** is decreased, the high-frequency loss

TABLE 1

| Type                     | exp | L*<br>D10<br>um | S*<br>D10<br>um | L*<br>D90<br>um | S*<br>D90<br>um | L*<br>D50<br>um | S*<br>D50<br>um | D*<br>L*D50/<br>S*D50<br>g/<br>cm <sup>3</sup> | L*/S*<br>Wt<br>Ratio | P*<br>Ad*<br>wt % | t/<br>cm <sup>2</sup> | Initial<br>Perm | Hc<br>A/m | Pcv* | Pcv** |       |
|--------------------------|-----|-----------------|-----------------|-----------------|-----------------|-----------------|-----------------|------------------------------------------------|----------------------|-------------------|-----------------------|-----------------|-----------|------|-------|-------|
| Case for comp-<br>arison | 1   | 22.60           | 1.66            | 52.20           | 5.58            | 33.50           | 3.21            | 10.44                                          | 5.66                 | 6:4               | 5                     | 0.5             | 28.5      | 7.88 | 31.8  | 701.4 |
| Other cases              | 2   | 17.88           | 1.66            | 42.90           | 5.58            | 28.80           | 3.21            | 8.97                                           | 5.63                 | 6:4               | 5                     | 0.5             | 27.5      | 7.34 | 32.4  | 664.8 |
|                          | 3   | 10.16           | 1.66            | 36.25           | 5.58            | 20.40           | 3.21            | 6.36                                           | 5.62                 | 6:4               | 5                     | 0.5             | 26.2      | 8.01 | 36.1  | 643.8 |
|                          | 4   | 8.90            | 1.66            | 31.07           | 5.58            | 17.60           | 3.21            | 5.48                                           | 5.38                 | 6:4               | 5                     | 0.5             | 21.8      | 8.31 | 42    | 607.5 |

The experiment II shows an optimum weight ratio and D50 ratio between the first magnetic powder **10** and the second magnetic powder **20** as described above.

The Table 2 shows the magnetic body **40** made according to one embodiment of the present invention, wherein the weight ratio and the D50 ratio between the first magnetic powder **10** and the second magnetic powder **20** are illustrated along with other characteristics of magnetic body **40**.

can still be reduced. Based on the experiment II, one can find an optimum combination of the D50 ratio and the weight ratio between the first magnetic powder **10** and second magnetic powder **20**; and even if the particles of the first magnetic powder **10** and second magnetic powder **20** become smaller, the permeability can be kept constant while reducing the energy loss at both high and low-frequency bands.

TABLE 2

| Type                     | exp | L*<br>D10<br>um | S*<br>D10<br>um | L*<br>D90<br>um | S*<br>D90<br>um | L*<br>D50<br>um | S*<br>D50<br>um | D*<br>L*D50/<br>S*D50<br>g/<br>cm <sup>3</sup> | L*/S*<br>Wt<br>Ratio | P*<br>Ad*<br>wt % | t/<br>cm <sup>2</sup> | Initial<br>Perm | Hc<br>A/m | Pcv* | Pcv** |       |
|--------------------------|-----|-----------------|-----------------|-----------------|-----------------|-----------------|-----------------|------------------------------------------------|----------------------|-------------------|-----------------------|-----------------|-----------|------|-------|-------|
| Case for comp-<br>arison | 1   | 22.6            | 1.66            | 52.2            | 5.58            | 33.5            | 3.21            | 10.44                                          | 5.66                 | 6:4               | 5                     | 0.5             | 28.5      | 7.88 | 31.8  | 701.4 |
| Other cases              | 1-1 | 22.6            | 1.66            | 52.2            | 5.58            | 33.5            | 3.21            | 10.44                                          | 5.5                  | 7:3               | 5                     | 0.5             | 25.9      | 8.22 | 33.7  | 716.7 |
|                          | 2   | 17.88           | 1.66            | 42.9            | 5.58            | 28.8            | 3.21            | 8.97                                           | 5.63                 | 6:4               | 5                     | 0.5             | 27.5      | 7.34 | 32.4  | 664.8 |
|                          | 3   | 10.16           | 1.66            | 36.25           | 5.58            | 20.4            | 3.21            | 6.36                                           | 5.62                 | 6:4               | 5                     | 0.5             | 26.3      | 8.01 | 36.1  | 643.8 |
|                          | 3-1 | 10.16           | 1.66            | 36.25           | 5.58            | 20.4            | 3.21            | 6.36                                           | 5.66                 | 7:3               | 5                     | 0.5             | 27.7      | 7.67 | 33    | 629   |
|                          | 4   | 8.9             | 1.03            | 31.07           | 5.58            | 17.6            | 3.21            | 5.48                                           | 5.38                 | 6:4               | 5                     | 0.5             | 21.8      | 8.31 | 42    | 607.5 |
|                          | 4-1 | 8.9             | 1.03            | 31.07           | 5.58            | 17.6            | 3.21            | 5.48                                           | 5.54                 | 7:3               | 5                     | 0.5             | 26.7      | 7.7  | 34.2  | 625.2 |

## 11

The following describes how to improve the initial permeability of the magnetic body made of amorphous alloy powder according to one embodiment of the present invention.

Table 3 shows test results of the magnetic body **40** made by using a mixture of the soft magnetic material **M** with different weight percentage of the adhesive material **30**, or different D50 of the second magnetic powder **20**, or different pressures for molding the magnetic body **40**, so as to increase the density and improve the initial permeability of the magnetic body **40**.

According to the aforementioned experiments experimental results, through the adjustment of the weight ratio and D50 ratio of the first magnetic powder **10** and the second magnetic powder **20**, the density of the magnetic body **40** can be increased, but the highest initial permeability reaches only about 28. Accordingly, the present invention proposes a way to further enhance the initial permeability by reducing the weight percentage of the adhesive material **30** in the mixture of the soft magnetic material **M** or adjusting the molding pressure to a range from 0.5 t/cm<sup>2</sup> to 1 t/cm<sup>2</sup> to reduce the spaces or gaps between the magnetic powders, so that the density of the magnetic body **40** and the initial permeability can be further enhanced.

The experimental results are shown in Table 3, when the molding pressure is from 0.5 tons per square centimeter to one ton per square centimeter, the density of the magnetic body **40** can be increased from 5.66 g/cm<sup>3</sup> to 5.68 g/cm<sup>3</sup>, and the initial permeability increase of 3 to 7% while the energy loss Pcv at lower frequencies (100 KHz/20 mT) has no significant change, but the energy loss at the high frequencies has an about 7 to 10 percent increase by the increased eddy current loss as the spaces or gaps between the magnetic particles decreased.

TABLE 3

| Type                        | exp | L*<br>D10<br>um | S*<br>D10<br>um | L*<br>D90<br>um | S*<br>D90<br>um | L*<br>D50<br>um | S*<br>D50<br>um | L*D50/<br>S*D50 | D*<br>g/<br>cm <sup>3</sup> | L*/S*<br>Wt/<br>Ratio | P*<br>t/<br>cm <sup>2</sup> | Initial<br>Perm | Hc<br>A/m | Pcv* | Pcv** |       |
|-----------------------------|-----|-----------------|-----------------|-----------------|-----------------|-----------------|-----------------|-----------------|-----------------------------|-----------------------|-----------------------------|-----------------|-----------|------|-------|-------|
| Case for<br>comp-<br>arison | 1   | 22.6            | 1.66            | 52.2            | 5.58            | 33.5            | 3.21            | 10.44           | 5.66                        | 6:4                   | 5                           | 0.5             | 28.5      | 7.88 | 31.8  | 701.4 |
| Other cases                 | 1-2 | 22.6            | 1.66            | 52.2            | 5.58            | 33.5            | 3.21            | 10.44           | 5.68                        | 6:4                   | 5                           | 1               | 30.5      | 8.69 | 32.1  | 769.6 |
|                             | 3-1 | 10.16           | 1.66            | 36.25           | 5.58            | 20.4            | 3.21            | 6.36            | 5.66                        | 7:3                   | 5                           | 0.5             | 27.7      | 7.67 | 33    | 629   |
|                             | 3-2 | 10.16           | 1.66            | 36.25           | 5.58            | 20.4            | 3.21            | 6.36            | 5.68                        | 7:3                   | 5                           | 1               | 28.6      | 8.2  | 32.5  | 671.2 |
|                             | 5   | 1.03            | 1.66            | 31.07           | 3.54            | 17.6            | 1.5             | 11.73           | 5.64                        | 7:3                   | 5                           | 0.5             | 29.4      | 6.09 | 25.9  | 520.9 |
|                             | 6   | 1.03            | 1.66            | 31.07           | 3.54            | 17.6            | 1.5             | 11.73           | 5.68                        | 7:3                   | 5                           | 1               | 30.7      | 7.02 | 27.9  | 606.9 |

In order to achieve a lower energy loss and a higher initial permeability at the same time, the D50 of the second magnetic powder **20** or the weight percentage of the adhesive material **30** are adjusted. As shown in Table 3, the initial permeability in the case 5 and case 6 has increased to 29 to 30. The energy loss at lower frequencies or high frequencies is lowest among all the cases. By doing so, the magnetic body **40** can be used to produce an inductor with higher Q factor. FIG. 7 shows the Q factor vs the frequencies of an inductor made by the present invention compared with conventional technology. As shown in FIG. 7, a peak Q factor of the inductor is greater than 50 at a frequency below 5 MHz.

FIG. 8 shows the inductance vs the frequencies of the inductor made by the present invention compared with conventional technology. As a result, the inductor made by the molding body produced in case 6 has achieved a higher

## 12

inductance compared with the conventional technology such as inductors made from Japanese inductor industries.

Although the present invention has been described with reference to the above embodiments, it will be apparent to one of ordinary skill in the art that modifications to the described embodiment may be made without departing from the spirit of the invention. Accordingly, the scope of the invention will be defined by the attached claims not by the above detailed descriptions.

What is claimed is:

1. A magnetic powder for mixing with a corresponding magnetic powder to make a magnetic body, wherein each of said magnetic powder and said corresponding magnetic powder is made of a soft magnetic material, and the average particle diameter of said magnetic powder is greater than that of said corresponding magnetic powder, wherein the ratio of the D50 of said magnetic powder to the D50 of said corresponding magnetic powder is in the range of 5 to 12, wherein said magnetic powder weighs 50 to 90 percent of the total weight of said magnetic powder and said corresponding magnetic powder weighs 10 to 50 percent of the total weight of said magnetic powder and said corresponding magnetic powder, wherein the D50 of said magnetic powder is in the range of 17 to 36 um, the D10 of said magnetic powder is in the range of 8 to 26 um, and the D90 of said magnetic powder is in the range of 30 to 52 um, for pairing with a corresponding D50, D10 and D90 of said corresponding magnetic powder to increase the density of the magnetic body.

2. The magnetic powder according to claim 1, wherein each of said magnetic powder and said corresponding magnetic powder is made of amorphous alloy.

3. The magnetic powder according to claim 1, wherein said magnetic powder weighs 60 to 80 percent of the total weight of said magnetic powder and said corresponding magnetic powder weighs 20 to 40 percent of the total weight of said magnetic powder and said corresponding magnetic powder.

4. The magnetic powder according to claim 1, wherein said magnetic powder weighs 60 to 70 percent of the total weight of said magnetic powder and said corresponding magnetic powder weighs 30 to 40 percent of the total weight of said magnetic powder and said corresponding magnetic powder.

5. The magnetic powder according to claim 1, wherein the D50 of said magnetic powder is in the range of 20 to 34 um and the D50 of said corresponding magnetic powder is in the range of 1.8 to 3.2 um.

## 13

6. The magnetic powder according to claim 1, wherein the D50 of said magnetic powder is in the range of 17 to 20 um and the D50 of said corresponding magnetic powder is in the range of 1.0 to 1.8 um.

7. The magnetic powder according to claim 1, wherein the ratio of the D50 of said magnetic powder to the D50 of said corresponding magnetic powder is in the range of 6 to 9.

8. The magnetic powder according to claim 1, wherein the ratio of the D50 of said magnetic powder to the D50 of said corresponding magnetic powder is in the range of 10 to 12.

9. The magnetic powder according to claim 1, wherein each of said magnetic powder and said corresponding magnetic powder is made of iron powders.

10. The magnetic powder according to claim 1, wherein said magnetic powder is made of amorphous alloy powder, wherein said magnetic powder comprises 0.5~1 wt % C, 6.2~7.2 wt % Si, 0~3.0 wt % Cr, 2.2~2.8 wt % B, and the rest is Fe, wherein 0% is less than 5000 ppm.

11. The magnetic powder according to claim 1, wherein the ratio of the number of particles of said magnetic powder at D50 to the number of particles of said magnetic powder at D10 is greater than 2, and the ratio of the number of particles of said magnetic powder at D50 to the number of particles of said magnetic powder at D90 is greater than 1.

12. The magnetic powder according to claim 1, wherein the ratio of the number of particles of said magnetic powder at D50 to the number of particles of said magnetic powder at D10 is greater than 3, and the ratio of the number of particles of said magnetic powder at D50 to the number of particles of said magnetic powder at D90 is greater than 1.5.

13. A method for making a magnetic body, said method comprising:

forming a first magnetic powder;

forming a second magnetic powder, wherein each of the first magnetic powder and the second magnetic powder is made of a soft magnetic material, and the average particle diameter of the first magnetic powder is greater than that of the second magnetic powder, wherein the ratio of the D50 of the first magnetic powder to the D50 of the second magnetic powder is in the range of 5 to 12, wherein the first magnetic powder weighs 50 to 90 percent of the total weight of the first magnetic powder and the second magnetic powder, and the second magnetic powder weighs 10 to 50 percent of the total weight of the first magnetic powder and the second magnetic powder; and

mixing the first magnetic powder and the second magnetic powder for making the magnetic body, wherein the D50 of the first magnetic powder is in the range of 17 to 36 um, the D10 of the first magnetic powder is in the range of 8 to 26 um, and the D90 of the first magnetic powder is in the range of 30 to 52 um, for pairing with a

## 14

corresponding D50, D10 and D90 of the second magnetic powder to increase the density of the magnetic body.

14. The method according to claim 13, wherein each of the first magnetic powder and the second magnetic powder is made of amorphous alloy.

15. The method according to claim 13, wherein the ratio of the D50 of the first magnetic powder to the D50 of the second magnetic powder is in the range of 6 to 9.

16. The method according to claim 13, wherein the ratio of the number of particles of the first magnetic powder at D50 to the number of particles of the first magnetic powder at D10 is greater than 2, and the ratio of the number of particles of the first magnetic powder at D50 to the number of particles of the first magnetic powder at D90 is greater than 1.

17. The method according to claim 13, wherein the ratio of the number of particles of the first magnetic powder at D50 to the number of particles of the first magnetic powder at D10 is greater than 3, and the ratio of the number of particles of the first magnetic powder at D50 to the number of particles of the first magnetic powder at D90 is greater than 1.5.

18. The method according to claim 13, wherein each of the first magnetic powder and the second magnetic powder is made of iron powders.

19. An electronic device, comprising:

a magnetic body, comprising:

a first magnetic powder; and

a second magnetic powder, mixed with the first magnetic powder, wherein each of the first magnetic powder and the second magnetic powder is made of a soft magnetic material, and the average particle diameter of the first magnetic powder is greater than that of the second magnetic powder, wherein the ratio of the D50 of the first magnetic powder to the D50 of the second magnetic powder is in the range of 5 to 12, wherein the first magnetic powder weighs 50 to 90 percent of the total weight of the first magnetic powder and the second magnetic powder, and the second magnetic powder weighs 10 to 50 percent of the total weight of the first magnetic powder and the second magnetic powder, wherein the D50 of the first magnetic powder is in the range of 17 to 36 um, the D10 of the first magnetic powder is in the range of 8 to 26 um, and the D90 of the first magnetic powder is in the range of 30 to 52 um, for pairing with a corresponding D50, D10 and D90 of the second magnetic powder to increase the density of the magnetic body; and

a wire, disposed in the magnetic body.

20. The electronic device according to claim 19, wherein the electronic device is an inductor.

\* \* \* \* \*